

## UNITED STATES PATENT OFFICE

2,673,164

PROCESS OF TREATING ASPHALT TO  
IMPROVE ITS ADHESION

Everett C. Hughes, Shaker Heights, and Harrison M. Stine, East Cleveland, Ohio, assignors to The Standard Oil Company, Cleveland, Ohio, a corporation of Ohio

No Drawing. Application August 1, 1950,  
Serial No. 177,134

6 Claims. (Cl. 106—273)

1

The present invention relates to a process for preparation of asphalt-containing compositions of improved adhesive properties, and more particularly to a process for combining asphalt with the reaction product of a phosphorus sulfide and water, and to the asphalt-containing reaction product obtainable by said process.

The term "asphalt" as used herein is applied to an asphalt suitable for direct use in highway work, roofing, and also for other purposes and includes asphalts brought to a consistency desired for a particular use, either by distillation or by mixing or fluxing with a harder or a softer asphalt, as the case may be. The term includes natural asphalt, such as asphaltic rocks, tars and pitches obtained in the distillation of coal or wood, petroleum residues, cracking coal tars, etc. The invention is particularly adapted for use with asphalt from petroleum sources which is commonly known as "asphalt cement." Asphalt cement is a highly viscous product obtained by oxidizing or steam-blowing a petroleum residue to increase its penetration, and the term is used to distinguish from such a product which is diluted or cut back with a solvent or emulsified with water.

The ability of the asphalt material in bituminous road matte to resist the action of water is an important factor in determining the service life of the road's surface. Unless the asphalt material shows a strong adhesion to aggregate, heavy rains penetrating the matte selectively wet the aggregate and thereby wash the aggregate free of asphalt; this eventually tears the pavement apart. If the adhesion of asphalt to aggregate were raised to a point above that of water to aggregate, the preferential wetting which leads to stripping could be prevented and a considerable saving would result.

Moreover, predrying the aggregate before laying the pavement could be avoided. In most bituminous road construction it is undesirable to remove all water from aggregate so as to obtain strong adhesion when the pavement is initially laid, because this is an expensive time-consuming process. If the asphalt-aggregate adhesion were much greater than the water-aggregate adhesion, the asphalt would force the water from the aggregate surface, selectively displacing it, so that wet aggregate would be as amenable to paving as dry aggregate.

Many approaches to this problem have been employed by the art, but with indifferent success. Each method has attacked the problem by seek-

2

ing to modify the wetting properties of either the asphalt or the aggregate.

In one method the wetting characteristics of the asphalt and aggregate are altered by treatment thereof with water-soluble detergents or wetting agents. A large number of materials have been suggested for this purpose, including sulfuric acid or aryl sulfonic acid esters of lower primary alcohols, sulfur compounds, wax, tall oil and oil-soluble water-insoluble heavy metal salts.

In another procedure, addition agents, usually termed additives, are incorporated in the asphalt in order to improve its wetting properties. A number of such additives have been recommended in the patent literature, including fats, fatty acids, heavy metal soaps, oleylamine, waxes, and synthetic or organic compounds having detergent or wetting properties.

However, surface-active agents have in general been found to be quite specific, both with respect to the asphalt material employed and to the nature of the aggregate surface. A large variety of chemically different surfaces are encountered in the average commercial aggregate, and thus such selective action is quite disadvantageous. The use of such agents has therefore not proved to be a practical expedient.

Moreover, if these compounds are water-soluble, they have the further disadvantage that they are leached out in time by rain which penetrates the pavement, and after they have been lost the adhesive properties of the asphalt and/or aggregate return to their original value. On the other hand, when the compounds are water-insoluble, the increase in adhesion is not as effective as might be desired.

Accordingly, it is an object of the present invention to provide a process for increasing the adhesion of asphalt to aggregate.

It is a further object of the invention to combine asphalt with an additive in order to permanently increase the adhesion thereof to aggregate without danger of loss of the additive in service.

It is a further object of the invention to provide a process for producing asphalt which may be used with water-wet aggregate in road mix construction, thereby avoiding the need for predrying the aggregate.

It is a further object of the invention to provide a process for improving the adhesion of asphalt to aggregate that is simple to employ and commercially feasible.

The adhesion of asphalt to aggregate can be evaluated by the Ohio State Department of High-

ways Supplemental Specification Test M-205.1, known as The Ohio Test.

In this test the asphalt is evaluated as follows: 100 grams of standard reference stone composed of 50% silica gravel and 50% crushed limestone graded to pass a  $\frac{3}{8}$  inch sieve and to be retained on a  $\frac{1}{4}$  inch sieve is dried one-half hour at 275° F. and coated with 5 grams of asphalt by mixing with a spatula for three minutes. The mixture is spread thinly on a plate and allowed to cure at a laboratory temperature for one hour. The mixture is then immersed in distilled water at 180° F. for one half hour, after which the number of particles showing stripping is determined. In order to pass the test, the material must show a coating value of at least 95%, i. e., a stripping from not over 5% of the aggregate particles.

In a variation of the Ohio test, the mixture is immersed in distilled water at 212° F. instead of 180° F. for one-half hour. This is a more rigorous test than the regular Ohio test.

Asphalts prepared in accordance with this invention are evaluated by either the Ohio test or the above-described variation thereof.

In accordance with this invention, asphalt which does not meet adhesion requirements of the Ohio test is combined with the reaction product of a phosphorus sulfide and water at a temperature and for a time sufficient to bring the asphalt to an adhesion within the requirements of the said test.

It will be perceived that the objects achieved in accordance with the invention include the provision of economic asphalts of highest quality and their preparation by combining a lower quality asphalt with an additive comprising the reaction product of a phosphorus sulfide and water in an amount to bring the adhesion of the asphalt up to the desired quality standard.

Among the phosphorus sulfides which may be reacted with water to produce the additive reacted with asphalt in accordance with the invention are tetraphosphorus trisulfide,  $P_4S_3$ , tetraphosphorus pentasulfide,  $P_4S_5$ , tetraphosphorus heptasulfide,  $P_4S_7$ , triphosphorus hexasulfide,  $P_3S_6$ , and phosphorus pentasulfide,  $P_2S_5$ . Each of these compounds reacts with water to produce a complex solution containing a large number of reaction products of wide variety.

The reaction product is formed by combining one mole of the phosphorus sulfide with from  $\frac{1}{2}$  to 4 moles of water, preferably two moles of water, and then heating the mixture at a temperature in the range of 150° to 350° F. for from  $\frac{1}{2}$  to 10 hours, the lower the temperature the longer the time and vice-versa. It is beneficial to carry out the reaction in a closed container under pressure of the gases formed in the course of the reaction, principally hydrogen, phosphine and hydrogen sulfide, but this is not essential. Pressure may be maintained at any desired value, say 70 pounds per square inch, by bleeding off the gases that are formed.

For example, a suitable additive may be prepared from phosphorus pentasulfide by reacting one mole thereof with two moles of water at 250° F. for one hour, maintaining the pressure at 70 pounds per square inch by bleeding off the hydrogen sulfide formed. The reaction product formed by this process is a liquid which has the approximate empirical formula  $PaS_3O_2$  and is a complex and unique mixture of known and unknown phosphorus and sulfur derivatives in unknown proportions.

Instead of employing water it is also possible to employ dilute aqueous acid solution, such as

may be formed by dissolving sulfuric, hydrochloric or phosphoric acid in water, or dilute aqueous alkali solution, such as may be formed by dissolving sodium hydroxide, calcium oxide or hydroxide or potassium hydroxide in water. All of the above are included in the expression "aqueous solution."

The additive prepared as described is blended with the asphalt in an amount in the range of from 0.1 to 2.0% and the resulting mixture heated at a temperature and for a time sufficient to bring the asphalt to an adhesion within the requirements of the Ohio test. The amount depends in part on the asphalt and on the conditions used in preparing the additive.

It has been found in accordance with the invention that maintenance at a temperature in the range of 212 to 500° F. for from 4 to 400 hours, the lower the temperature the longer the time and vice-versa, will increase the adhesion of an asphalt which does not meet the Ohio test 95% adhesion requirement to a value within this requirement. If a temperature in the range of 300 to 450° F. and a combining time of 12 to 100 hours are employed, the asphalt will have an adhesion of from 98 to 100% in the Ohio test, and therefore these conditions are preferred. There is no upper limit to the heating time since after the period has elapsed there is no objection to longer heating.

The additive may be used in any amount that will result in the desired improvement. Generally, the amount falls within the range of 0.1% to 2%, usually 0.25% to 1.0%.

The following examples are of interest in connection with the various methods of preparing the improved asphalt in accordance with the invention.

#### Example 1

One mole of phosphorus pentasulfide was reacted with one mole of water at 200° F. for 2 hours, at atmospheric pressure. This additive in the amount of 0.25% by weight was added to asphalt from a Mid-Continent crude and the mixture then heated at 300° F. in an atmosphere of carbon dioxide for 336 hours. A 100 gram sample of the reaction product was tested by the Ohio test and a coating value of 100% obtained.

#### Example 2

One mole of phosphorus pentasulfide was reacted with two moles of water at 250° F. for one hour, maintaining the pressure at 70 pounds per square inch by bleeding off the hydrogen sulfide formed. This additive in an amount of 0.5% by weight was added to asphalt from a Mid-Continent crude and then tested by the variation of the Ohio test in which the stripping water bath is maintained at 212° F. instead of 180° F. for one-half hour. The coating value was 88%.

The mixture was then heated for 24 hours at 300° F. in an atmosphere of carbon dioxide. At the end of this time the coating value was increased to 94% as measured by the same test. After heating the mixture for an additional 72 hours at 300° F. the coating value was 98%.

The results show that the improved result obtained in accordance with the invention is developed only after reaction between the additive and the asphalt, and further that the minimum reaction time at 300° F. is approximately 24 hours.

In contrast, a sample of the asphalt which did not contain an additive gave a value of 65% by the same variation of the Ohio test before heat-

ing. This value decreased to 55% after heating for 24 hours and then increased slightly to 60% after an additional heating for 72 hours at 300° F.

In the above examples the blanket of carbon dioxide is employed to prevent further oxidation of the asphalt with a consequent decrease in its penetration. There is no objection to the heating in an atmosphere of air where the decrease in penetration is not important, or where the surface of the asphalt exposed to air is small compared to the volume so there is a minimum of oxidation.

The nature of the action which takes place during the process of the invention is unknown. However, the adhesion of the asphalt is increased considerably, as the data in the examples show, while the penetration of the asphalt falls slightly. The latter result is not a disadvantage for it may be overcome by use of an asphalt having a somewhat higher penetration than it is desired to employ finally.

In the Ohio test the aggregate used is dry. It will, however, be obvious that the invention is not limited to an asphalt to be used on dry stone since the adhesion of the asphalt is improved to such an extent that it will adhere to wet stone or any other surface to be coated with asphalt, such as wood, paper, roofing material, concrete, etc.

It will be noted that there are a number of variables in making the initial phosphorus sulfide-water reaction product and also in making the final asphalt-additive reaction product. These are defined as covering relatively wide ranges, while variations within these ranges result in additives and asphalt compositions of somewhat different properties. They are all effective for improving the adhesion of asphalt, and none of the variables are critical in this regard.

It will be obvious that in view of the many variables entering into the process by which the additive-asphalt reaction product is made there are many variations falling within the invention that are not included in the illustrative examples. It is intended that all of these variations are included as fall within the following claims.

All parts and percentages in the specification and claims are by weight.

The term "consisting essentially of" does not exclude ingredients which do not change the character of the asphalt composition or ingredients which are essential to the composition. The term thus excludes phosphorus sulfide-olefin-water reaction products.

We claim:

- 10 1. A process of preparing an asphalt composition having improved adhesion to aggregate which comprises adding to an asphalt a small amount of an additive consisting essentially of the reaction product of a phosphorus sulfide and an aqueous solution, reacted under non-oxidizing conditions, and heating the mixture of asphalt and additive at a temperature between about 212° and 500° F. for a time of at least 4 hours to improve the adhesion of the asphalt to aggregate.
- 15 2. The process of claim 1 in which the phosphorus sulfide is phosphorus pentasulfide.
- 20 3. A process in accordance with claim 1 wherein the additive is employed in an amount within the range of 0.1 to 2%.
- 25 4. An asphalt obtained by the process of claim 1.
- 30 5. An asphalt in accordance with claim 4 in which the phosphorus sulfide is phosphorus pentasulfide.
- 35 6. The asphalt of claim 4 wherein the asphalt comprises from 0.1 to 2% of the reaction product of phosphorus sulfide and water.

EVERETT C. HUGHES.  
HARRISON M. STINE.

References Cited in the file of this patent

UNITED STATES PATENTS

| 40 | Number    | Name      | Date           |
|----|-----------|-----------|----------------|
|    | 1,054,250 | Stock     | Feb. 25, 1913  |
|    | 2,093,450 | Jacobsohn | Sept. 21, 1937 |
|    | 2,450,756 | Hoiberg   | Oct. 5, 1948   |
|    | 2,534,217 | Bartleson | Dec. 19, 1950  |

FOREIGN PATENTS

| Number  | Country | Date         |
|---------|---------|--------------|
| 420,832 | France  | Feb. 8, 1911 |